

# UNITED STATES PATENT OFFICE.

JACOB BREDEL, OF HÖCHST-ON-THE-MAIN, GERMANY.

## MANUFACTURE OF ARTICLES FROM QUARTZ-GLASS.

No. 816,708.

Specification of Letters Patent.

Patented April 3, 1906.

Application filed September 19, 1904. Renewed August 30, 1905. Serial No. 276,478.

*To all whom it may concern:*

Be it known that I, JACOB BREDEL, a subject of the German Emperor, and a resident of Höchst-on-the-Main, Germany, have invented certain new and useful Improvements in and Relating to the Manufacture of Articles from Quartz-Glass, of which the following is a specification.

This invention has reference to improvements in and relating to the manufacture of articles from quartz-glass; and it consists in the improved manner or process of manufacture, substantially as hereinafter described.

If the raw material employed consists of rock crystal, broken quartz, or the like, this after being broken into small pieces is heated to a temperature of about 1,000° centigrade and then immediately thrown into cold water. If quartz-sand, silica, or the like be used, this is first melted at such a suitable temperature as to convert it into a homogeneous mass, which after being cooled is broken up into small pieces. These pieces are also heated to a temperature of about 1,000° centigrade and, like the broken quartz, quickly cooled in water. This heating and rapid cooling of the material is repeated, and the coefficient of expansion of the resultant material is thereby greatly diminished.

After the material has been treated as de-

scribed it is melted and brought to such a sufficiently high temperature that the metal becomes very fluid, after which a jet of hot air or steam is allowed to pass into it, which transforms the metal into a more or less fibrous or woolly form, the degree of fineness of the fibers depending upon the heat and consequent fluidity of the metal when subjected to the hot-air or steam jet. This resultant fibrous or woolly material is next 35 pressed or molded into the required form of the article to be made, and this is fused to make it revert into a homogeneous mass, the melting being begun preferably from the bottom, as by this means the formation of air- 40 bubbles is obviated. 45

Having now fully described my said invention, what I claim, and desire to secure by Letters Patent, is—

In the manufacture of articles from quartz-glass, first converting the raw material into a fibrous or woolly state and then after molding same into the required form again melting it, substantially as described. 50

In testimony whereof I have hereunto set 55 my hand in presence of two witnesses.

JACOB BREDEL.

Witnesses:

JEAN GRUND,  
CARL GRUND.